

# United States Patent

[19]

Miller et al.

[11] 3,884,820

[45] May 20, 1975

[54] GREASE COMPOSITION

[75] Inventors: **James E. Miller**, Griffith; **Reuben A. Swenson**, Whiting, both of Ind.

[73] Assignee: **Standard Oil Company**, Chicago, Ill.

[22] Filed: **Apr. 19, 1971**

[21] Appl. No.: **135,473**

[52] U.S. Cl. .... **252/41; 252/59**

[51] Int. Cl. .... **C10m 5/14; C10m 5/10**

[58] Field of Search..... **252/41, 59, 39**

[56] References Cited

UNITED STATES PATENTS

2,627,938 2/1953 Frohmader et al. .... **252/59**  
2,833,718 5/1958 Morway et al. .... **252/39**  
3,083,160 3/1963 Agius et al. .... **252/29**

3,271,311 9/1966 Morway et al. .... **252/41**  
3,290,244 12/1966 Polishuk et al. .... **252/41**  
3,293,179 12/1966 Bertocsk ..... **252/41**  
3,396,108 8/1968 Caruso..... **252/18**

Primary Examiner—Delbert E. Gantz

Assistant Examiner—I. Vaughn

Attorney, Agent, or Firm—Edwin C. Lehner; Arthur G. Gilkes; William T. McClain

[57] ABSTRACT

A mineral oil grease which is resistant to separation by centrifugal force is provided by using as the sole thickening agent either polyethylene having a number average molecular weight of from about 1,500 to about 3,000 or a combination of said polyethylene with a small amount of a lithium higher fatty acid soap.

10 Claims, No Drawings

## GREASE COMPOSITION

## BACKGROUND OF THE INVENTION

## 1. Field of the Invention

This invention relates to grease compositions which are resistant to separation of the thickening agent from the base lubricating oil during use under centrifugal force conditions.

## 2. Description of the Prior Art

Large rotary compressors, operating at speeds from in the range of 5,000 to about 15,000 rpm, are well-known devices used in the gas compression art. Coupling of the drive shafts of the rotary compressor and prime mover, such as a steam turbine, is effected by means of high speed flexible gear couplings which are provided with gears for vertical and lateral movement during operation. Lubrication of such gear couplings is extremely important because such compressors are continuously operated for extended periods of time. The use of sealed couplings to permit the use of liquid lubricating oils as the lubricant is not satisfactory because of alignment problems between the driving and driven shafts. Maintenance of the liquid seal under misalignment conditions is therefore extremely difficult. Consequently, most of the gear couplings now in use are of the unsealed type which require the use of a grease as the lubricant. A grease suitable for this latter type of high speed coupling lubrication needs to be heavy enough to be packed into the couplings by hand and be able to lubricate the coupling satisfactorily for periods of many months of continuous operation. Conventional greases, i.e., greases thickened by metal soaps and solid fillers, such as graphite and molybdenum disulfide, separate into their components in this service and frequent replacement is required, sometimes as often as every three months. Thus, a grease is needed that will not separate under the centrifugal forces developed in the operation of the aforesaid high speed flexible gear couplings.

## SUMMARY OF THE INVENTION

It has been discovered that low molecular weight polyethylene can be used either alone or in combination with a small amount of lithium soap as the sole thickening agent for mineral lubricating oil to form greases which are resistant to centrifugal separation and suitable for use as the lubricant for unsealed high speed flexible gear couplings.

Commercially available low molecular weight polyethylenes suitable for use in the present invention have a number average molecular weight in the range of from about 1,500 to about 3,000, preferably 2,000, and a melting or softening point in the range of from about 210° to about 240°F.

The greases of the present invention consist essentially of a mineral lubricating oil having a viscosity in the range of from about 130 to about 200 SSU at 210°F containing as the sole thickening agent for said oil either (a) from about 6 to about 10, preferably 7 - 8, weight per cent of polyethylene having a number average molecular weight in the range of from about 1,500 to about 3,000, preferably about 2,000, or (b) from about 6.5 to about 12 weight per cent of a mixture consisting of (i) from about 6 to about 10 weight per cent of polyethylene having a number average molecular weight in the range of from about 1,500 to about 3,000 and (ii) from about 0.5 to about 2, preferably about

0.85 to about 0.9, weight per cent of a lithium soap. Greases formed with the polyethylene alone have a drop point of about 140° to about 160°F. Since the operating temperatures of the couplings are generally within the range of about 150° to about 200°F, it is desirable to improve the thermal stability of the centrifugally stable greases of this invention. It has been discovered that, when a small amount of a conventional lithium soap grease thickener is incorporated with the aforesaid polyethylene during the manufacture of the grease of this invention, the drop point of the resultant grease is raised to above 200°F without adversely affecting the centrifugal stability of the grease. The greases of this invention initially have an NGLI (National Lubricating Grease Institute) grade consistency of about 3 or 4 and after working will have an NGLI grade of about 0 to 1. This softening characteristic of the grease is highly desirable for it can be easily handled during packing of the couplings and thereafter satisfactorily lubricate the gear couplings at their operating temperatures without separation of its components and thus provide extended operation of the gear couplings without any loss in lubrication.

The mineral lubricating oil used in the greases of this invention can be any of the conventional petroleum lubricating oils having a viscosity in the range of about 130 to about 200 SSU (Saybolt Seconds Universal) at 210°F. A preferred petroleum lubricating oil is a bright stock having a viscosity of about 180 - 195 SSU at 210°F.

The lithium soap employed in the present invention is well known in the art. The term "lithium soap" used herein and in the claims refers to the soaps or salts which are formed by the reaction of lithium hydroxide with fats or higher fatty acids such as stearic, hydroxystearic, palmitic, oleic and the like. In place of the substantially pure fats or acids, mixtures of fats or fatty acids such as those obtained from the various fatty oils such as cotton seed oil, rapeseed, mineral oils, fish oils and the like can be used. The saturated fatty acids such as those derived from hydrogenated oils of vegetable, animal and marine origin can also be used. A preferred lithium soap is the lithium salt of a mixture of hydrogenated castor oil and hydrogenated fish oil fatty acids.

When desired, conventional grease additives such as extreme pressure agents, oxidation inhibitors, corrosion inhibitors and the like can be effectively incorporated in the grease compositions of this invention.

In preparing the greases of this invention, the polyethylene is simply added to the base lubricating oil at a temperature of about 250°F and held with agitation for a period of about 30 minutes to assure complete solution of the polymer in the oil. If the lithium soap is included, it is combined with the base oil prior to addition of the polyethylene to the heated oil. After the polyethylene is dissolved, the mixture is cooled to about 200°F and any supplementary additives such as extreme pressure agents, antioxidants and rust inhibitors are then incorporated. Thereafter, the mixture is cooled, with or without stirring, to about 175° - 190°F and packaged. No milling of the grease mixture is required to form the grease compositions of this invention.

## 65 DESCRIPTION OF THE PREFERRED EMBODIMENTS

Centrifugal stability of the greases described herein

was determined by centrifuging at 150°F a sample of the grease in a centrifuge operating at 4,300 rpm. The relative centrifugal force (RCF) imposed on the grease in this test is equivalent to 3,870 G. A gear coupling operating at 7,000 rpm has an RCF of about 3,700.

In the exemplary formulations set forth in the following Table, a conventional lithium soap grease, containing 7 percent lithium soap of hydrogenated castor oil and hydrogenated fish oil fatty acids (the ratio of castor oil to the fatty acid being 10), was used to provide the indicated amounts of lithium soap in the greases of this invention.

The low molecular weight polyethylene used in preparing the illustrative greases of this invention has a number average molecular weight of about 2,000 and a softening point of about 220°F and is available commercially under the trade name "A-C Polyethylene 6."

2. The composition of claim 1 wherein the molecular weight of said polyethylene is about 2,000.
3. The composition of claim 2 wherein said thickening agent is about 7 weight percent polyethylene.
5. 4. The composition of claim 2 wherein said thickening agent is a mixture of about 7 weight percent polyethylene and about 0.85 to about 0.9 weight percent lithium soap.
10. 5. The composition of claim 4 wherein said lithium soap is a lithium salt of a mixture of hydrogenated castor oil and hydrogenated fish oil fatty acids.
15. 6. In the operation of centrifugal gear couplings wherein a solid lubricant is used to lubricate the gears in said coupling, the improvement comprising using as said lubricant the grease composition of claim 1.
7. In the operation of centrifugal gear couplings wherein a solid lubricant is used to lubricate the gears

TABLE

| Ingredients*                | 1    | 2    | 3    | 4    | Formulation 5 | 6    | 7    |
|-----------------------------|------|------|------|------|---------------|------|------|
| Lubricating Oil**           | 86.5 | 87.6 | 89.6 | 60.0 | 67.0          | 75.0 | 74.0 |
| Lithium Soap Grease         | —    | —    | —    | 30.0 | 20.1          | 12.6 | 12.4 |
| Lithium Soap                | —    | —    | —    | 2.1  | 1.4           | 0.88 | 0.87 |
| "A-C 6" polyethylene        | 6.9  | 7.0  | 5.0  | 4.5  | 8.1           | 7.0  | 6.9  |
| Zinc dialkyldithiophosphate | 3.6  | 3.6  | 3.6  | 3.6  | 3.2           | 3.6  | 3.6  |
| Lead Naphthenate            | 1.8  | 1.8  | 1.8  | 1.8  | 1.6           | 1.8  | 1.8  |
| Ortholeum 300***            | 0.2  | —    | —    | —    | —             | —    | 0.2  |
| Phenyl-alpha-naphthylamine  | 0.1  | —    | —    | —    | —             | —    | 0.1  |
| Zinc naphthenate            | 1.0  | —    | —    | —    | —             | —    | 1.0  |
| Penetrations:               |      |      |      |      |               |      |      |
| Unworked                    | 194  | 198  | 425  | —    | 230           | 234  | 196  |
| Worked, 60 strokes          | 326  | 332  | 479  | 360  | 352           | 333  | 339  |
| NLGI Grade:                 |      |      |      |      |               |      |      |
| Unworked                    | 4    | 4    | —    | —    | 3             | 3    | 4    |
| Worked, 60 strokes          | 1    | 1    | —    | 0    | 0             | 1    | 1    |
| Hours Centrifuged           | 48   | 72   | —    | 24   | 72            | 72   | 48   |
| Oil Separation, wt. %       | 0    | 0    | —    | 4.5  | 0             | 0    | 0    |
| Drop Point, °F              | 145  | —    | —    | —    | —             | —    | 248  |

\* - In wt. %.

\*\* - Petroleum bright stock having a viscosity of 187 SSU at 210°F.

\*\*\* - Commercial antioxidant identified as a mixture of aromatic amines.

We claim:

1. A grease resistant to separation by centrifugal force consisting essentially of a mineral lubricating oil having a viscosity in the range of from about 130 to about 200 SSU at 210°F containing as the sole thickening agent for said oil either (a) from about 6 to about 10 weight per cent of polyethylene having a number average molecular weight in the range of from about 1,500 to about 3,000 or (b) from about 6.5 to about 12 weight per cent of a mixture consisting of (i) from about 6 to about 10 weight per cent of polyethylene having a number average molecular weight in the range of from about 1,500 to about 3,000 and (ii) from about 0.5 to about 2 weight per cent of a lithium higher fatty acid soap.

in said coupling, the improvement comprising using as said lubricant the grease composition of claim 2.

8. In the operation of centrifugal gear couplings wherein a solid lubricant is used to lubricate the gears in said coupling, the improvement comprising using as said lubricant the composition of claim 3.

50 9. In the operation of centrifugal gear couplings wherein a solid lubricant is used to lubricate the gears in said coupling, the improvement comprising using as said lubricant the composition of claim 4.

10. In the operation of centrifugal gear couplings wherein a solid lubricant is used to lubricate the gears in said coupling, the improvement comprising using as said lubricant the composition of claim 5.

\* \* \* \* \*